

July 16, 1929.

J. DUCLAUX

1,720,670

MANUFACTURE OF ULTRAFILTER MEMBRANES

Filed Aug. 30, 1923



Inventor  
Jacques Duclaux  
By Henry Orthofer  
Atty.

Patented July 16, 1929.

1,720,670

# UNITED STATES PATENT OFFICE.

JACQUES DUCLAUX, OF PARIS, FRANCE.

MANUFACTURE OF ULTRAFILTER MEMBRANES.

Application filed August 30, 1923, Serial No. 660,179, and in France September 11, 1922.

It is well known that membranes called ultra-filters comprising cellulose ester films, have been used for some years in scientific research laboratories. Several processes for 5 their preparation have been described, but these processes, which are suitable for laboratories, are too costly or too complicated to be of industrial application. They are not suited for use in preparing for instance, 10 several hundred square metres of ultra-filter membrane, as it is necessary to do in industrial operations.

The invention has for its object a process for the production of these membranes 15 in large quantities. This process has the advantage of being particularly economical owing to the fact that most of the solvent used for dissolving the cellulose ester can be recovered and used over again. The in- 20 vention also includes certain improved mem- branes of the type later described.

According to this invention I form the cellulose ester films constituting the ultra- 25 filter on an unrolling strip of smooth cloth which is guided by rollers so as to dip first into a solution of cellulose ester and subsequently into a coagulating liquid.

Referring to the appended drawing illustrating diagrammatically, as an example, 30 an apparatus for carrying out the process, the object of the invention.

The membrane, of cellulose ester and particularly of nitro cellulose, is forced upon 35 a strip of cloth of any length, carried on rollers. Starting from a first storage roll *a*, the band dips first into a trough *b* containing the solution of cellulose ester or collodion, then it passes upon a guiding roller *c* and issues vertically from the trough, carrying 40 by adhesion a certain quantity of collodion. At a certain distance above the trough, the strip of cloth, which has begun to dry, meets a system of rollers *d* and *e* which guide it through a vat *f* full of a coagulating 45 liquid, for instance, water, in which it proceeds for a while. It emerges from it completely hardened and freed from most of the solvent and is rolled up upon a last roll *g*.

50 In the example illustrated on the drawing, the strip passes only once in the vat filled with the coagulating liquid. It is evident, however, that it is possible, by means of other rollers, to lengthen its path in this liquid to ensure its more thorough washing. The single vat may also be replaced by sev-

eral successive vats, with a methodical circulation of coagulating liquid.

The speed of translation must be sufficiently slow for the collodion carried away 60 by the strip of cloth to be solidified before arriving at the roller *d* or else it might stick to the latter. For greater security, this roller may be covered with cloth, blotting paper or any other porous substance 65 impregnated with the coagulating solution; in this manner, adhesion is completely avoided, provided that the solution impregnating the roller is frequently renewed.

The recovery of the solvent of the cellulose ester may be effected in two ways. A first portion of this solvent evaporates during the passage of the cloth between the collodion trough *b* and the roller *d*. The vapours being heavier than air, fall vertically; it is sufficient to surround this part of the apparatus with a kind of casing and to collect at the lower portion the air loaded with vapours. Another portion of the solvent is carried by the cloth and is found dis- 80 solved in the coagulating liquid, from which it can be extracted.

It is possible to add to the machine so constructed an arrangement permitting the control of the uniformity of the membranes. It 85 suffices for this to add a coloring matter to the liquid contained in the coagulation vat. Variations in the texture or in the thickness of the filter membrane will then be represented by differences in coloration which 90 are at once perceptible.

In the method of manufacture of ultra- 95 filter membranes which has just been described, the strip of cloth acts merely as support of the cellulose ester film which is the filtering element that is to say the film is supported in and spans the open mesh of the weave. The passage of this strip of cloth in the collodion trough has simply for its object the impregnation of the cloth. It may 100 be replaced by any other arrangement conducive to the same result; for instance, the impregnation may be obtained in causing, by means of a nozzle, the collodion to flow on the cloth in a jet or thin film, either on 105 both sides or on one side only.

Before passing into the machine which impregnates it with collodion, the cloth strip may receive a preparation adapted to modify its filtering properties; it may for instance, be moistened with water or a solution having for its purpose to modify later on the 110

filtering properties of the cellulose ester film.  
I claim:

1. An ultra-filter membrane comprising a cloth with a nitrocellulose film adherent 5 thereto and filling the mesh thereof, said membrane being characterized by its method of manufacture, in that it is produced by impregnating cloth with a solution of nitrocellulose, the solvent of which is permitted 10 to evaporate until the film solidifies before the impregnated cloth is immersed in a coagulating bath.
2. The art of making ultra filter-mem- 15 branes which comprises passing cloth through a solution of nitrocellulose of a consistency that will adhere to the cloth and fill the mesh thereof, removing the cloth from said solution, permitting solvent to evapo- rate until the nitrocellulose coating has solid-

ified and the impregnated cloth does not ad- 20 here to a roller moistened with a coagulant for said nitrocellulose solution, and passing said cloth through a coagulating solution.

3. The art of making ultra-filter mem- 25 branes which comprises passing cloth through a solution of nitrocellulose of a consistency that will adhere to the cloth and fill the mesh thereof, removing the impregnated cloth from said solution, permitting solvent to evaporate until the nitrocellulose coating 30 has solidified and the impregnated cloth does not adhere to a roller moistened with water, and passing said cloth through water until the nitrocellulose coating has completely hardened.

In testimony that I claim the foregoing as my invention, I have signed my name.

JACQUES DUCLAUX.